

# UNITED STATES PATENT OFFICE.

RAYMOND F. BACON, OF PITTSBURGH, PENNSYLVANIA, ASSIGNOR TO METALS RECOVERY COMPANY, OF NEW YORK, N. Y., A CORPORATION OF MAINE.

## FLOTATION OF COAL.

1,329,493.

Specification of Letters Patent.

Patented Feb. 3, 1920.

No Drawing.

Application filed February 27, 1917. Serial No. 151,189.

To all whom it may concern:

Be it known that I, RAYMOND F. BACON, a citizen of the United States, residing at Pittsburgh, Allegheny county, State of Pennsylvania, have invented certain new and useful Improvements in Flotation of Coal; and I do hereby declare the following to be a full, clear, and exact description, such as will enable others skilled in the art 10 to which it appertains to make and use the same.

This invention relates to the concentration of bituminous coal by flotation, and particularly to the separation of such coal from slate and the like, and the separation of different grades or qualities of coal from each other.

The invention is based upon the discovery that when bituminous coal or coal refuse is 20 properly crushed and mixed with a small amount of oil or oil mixture or equivalent froth-forming agent the true coal substances can be floated and thereby removed from the slate and other constituents of a non-carbonaceous nature or even from other carbonaceous constituents than true coal substances.

The coal may be run of mine, or it may be coal refuse such as results, for example, 30 from coal washing processes, as well as culm coal or coal wastes of various kinds.

I have found it to be necessary, in the flotation of bituminous coal, to crush the coal or coal refuse to such an extent that 35 it will pass a 48 mesh or smaller sieve, in order to secure the maximum recovery of combustible matter. I have also found that it is necessary for the reduction of the coal or refuse to a fine form to be accomplished 40 in such a way that the resulting particles shall have sharp angular edges, in order to secure maximum recoveries; and I have further found that the rubbing or shearing action, such as is produced in a disk grinding machine, and which causes a rounding 45 of the particles of coal, inhibits the floating properties of the coal and at the same time increases the ash content of the concentrate. The grinding should accordingly be effected, for example, wet, as in a ball mill, or dry in any suitable form of grinding machine.

which does not subject the particles to a rounding action, in order to produce a material suitable for flotation.

When the material has been thus properly 55 ground, the combustible matter or free coal, both in run of mine bituminous coal and in mine or washer refuse or other waste coal material, can be more or less completely separated from the slate or other ash-forming material which it carries, as well as from certain undesirable pseudo coal constituents when present, by subjecting the finely divided material to a flotation operation. The flotation is effected by the use 65 of suitable oils or oil mixtures, such as coke-oven light oil, pine oil, "cold-weather mixture", petroleum, shale and coal oils, and other oils (mineral or vegetable) suitable for the purpose; or by the use of other appropriate frothing agents which enable a 70 proper froth to be produced. With certain flotation oils, acid or alkaline solutions of low concentration may also be employed advantageously, the effect being to improve 75 the quality or increase the quantity of floated coal. The flotation operation can be carried out in any appropriate type of apparatus, for example, a Callow pneumatic flotation cell.

The invention will be further illustrated by the following more detailed description of certain applications thereof:

The coal or coal refuse (washer waste, "bony" or mine waste) to be concentrated 85 is crushed to pass a 48-mesh sieve and thoroughly mixed with water (about 4 to 12 parts of water for each part of coal) and oil or oil mixture, etc., (0.5 to 3 lbs. per ton of coal). The resulting pulp is then transferred, for example, to a Callow pneumatic flotation cell and the air bubbles thereof, rising from the porous bottom of the cell, through the pulp, carry up with them the particles of free coal and appear on the surface 95 as an ephemeral foam which, constantly renewed, flows continuously over the cell wall into the launder. The foam or froth carries with it most of the combustible matter of the coal treated, whereas the tailings 100 are largely composed of non-combustible matter, the combustible matter present being

dependent upon the oil or like agent used and the pressure of the air supplied to the cell. Where it is desirable to add an acid or alkali or salt, the same can be added to the 5 water to produce, for example, a 0.1% solution or less, depending upon the requirements of the oil used.

The following are results obtained by the 10 treatment of coal material as described above using pine oil as the active frothing agent:

(1) A sample of bituminous coal washer refuse was crushed to pass a 48-mesh sieve, thoroughly mixed with four parts by weight 15 of water and pine oil in the proportion of about 1 lb. per ton of refuse, and floated in a Callow pneumatic flotation cell, collecting the froth which ran over the cell walls into the launder. The following results were obtained:

|                   | Ash. | Ash-free<br>coal. | Recover-<br>ery. |
|-------------------|------|-------------------|------------------|
| Concentrates..... | 25%  | 25%               | 25.53%           |
| Tailings.....     | 75%  | 80.35%            | 77.2%            |

(2) A similar treatment of the same material using 1.5 lbs. of pine oil per ton of refuse gave the following results:

|                   | Ash.  | Ash-free<br>coal. | Recover-<br>ery. |
|-------------------|-------|-------------------|------------------|
| Concentrates..... | 31.6% | 31.60%            | 21.6%            |
| Tailings.....     | 68.4% | 83.16%            | 89.6%            |

(3) A sample of run of mine bituminous coal was crushed to pass a 48 mesh sieve, thoroughly mixed with about four parts by weight of water, and pine oil in the proportion of 1 lb. per ton, and the material was floated in a Callow pneumatic flotation cell, collecting the froth which ran over the cell walls. The following results were obtained:

|                   | Ash.  | Ash-free<br>coal. | Recover-<br>ery. |
|-------------------|-------|-------------------|------------------|
| Concentrates..... | 94.8% | 7.91%             | 87.3%            |
| Tailings.....     | 5.2%  | 67.96%            | 97.9%            |

(4) A similar treatment of the same material using 12 parts of water to 1 of coal gave the following results:

|                   | Ash.  | Ash-free<br>coal. | Recover-<br>ery. |
|-------------------|-------|-------------------|------------------|
| Concentrates..... | 94.8% | 7.88%             | 87.3%            |
| Tailings.....     | 5.2%  | 66.58%            | 97.9%            |

The refuse and bituminous coal from 50 which the above results were obtained were found to have the following ash and free coal contents.

|                                              |        |
|----------------------------------------------|--------|
| Ash in refuse.....                           | 67.08% |
| Ash-free coal in refuse (by combustion)..... | 24.10% |
| Ash in coal.....                             | 10.84% |
| Ash-free coal in coal (by difference).....   | 89.16% |

As stated above, the nature and quantity of the coal floated is dependent upon the manner in which the coal has been ground 60 or crushed. The importance of proper crushing will be apparent from the following results obtained with two samples of the same coal refuse ground or crushed to substantially the same size and treated in the same manner with the same amount of oil. The

sample marked (1) was crushed to pass a 48-mesh sieve and showed particles with sharp angular edges and lustrous faces; while the sample marked (2) was passed through a disk grinding machine and 70 showed more or less rounded grains without marked luster the results being as follows:

|          | Concen-<br>trate. | Ash in<br>concen-<br>trate. | Ash<br>free<br>coal. | 75 |
|----------|-------------------|-----------------------------|----------------------|----|
| (1)..... | 7.5%              | 17.60%                      | 6.3%                 |    |
| (2)..... | 5.8%              | 36.32%                      | 3.7%                 |    |

Screen analyses of the two samples showed that they were not essentially different as regards size of particles. The importance of proper grinding, and the production of particles of proper character will thus be evident.

The concentration of coal by flotation, according to the present invention, enables coal constituents to be recovered from coal refuse 85 which is not commonly considered capable of further concentration by the usual methods of concentration. Thus the wastes from the washeries, containing the rejected material from the usual washing process, and 90 being relatively low in carbonaceous matter, can be effectively concentrated by the process of the present invention. Moreover, not only the common gangue constituents, but also the bony coal, slate, schist, shale, and 95 other non-carbonaceous or non-bituminous mineral substances can be separated from true coal substances.

The process of the present invention is moreover adapted for the reduction of the 100 ash content of run of mine coals, as a substitute for the ordinary washing processes, and other processes of concentration, for the separation of non-coal substances from true coals which are contaminated therewith. 105 Similarly the coal can be recovered from mine or washer wastes of all classes, including culm coal; and bituminous matter suitable for use as a fuel can be separated from coal mine or washer wastes of high 110 ash content, fuel material being thus produced from high ash substances. It is economically feasible, by the process of the present invention, to recover usable coals from present unusable wastes from coal 115 mines and washers. It is even possible to separate different coal constituents from each other in the manner above described.

The coal concentrate produced according to the present invention may be used directly as a boiler fuel, or it may be further pulverized, after drying, for use as powdered coal or for briquetting or coking and other purposes.

It will, of course, be evident that the same 125 water or acid or alkaline liquid utilized during the flotation can be separated from the tailings and used over again, where such use is desired. When the flotation process is operated in connection with coal washers, 130

the water accompanying the washer refuse may be utilized in the subsequent crushing and flotation operation, above described.

It is of great importance that the flotation of the comminuted finely-divided product should take place before the surfaces of the coal particles lose the physical characteristics imparted to them by the comminuting operation. For this reason if the comminution is effected while the coal is dry, the flotation should preferably follow immediately, or at least before atmospheric or other influences materially dull or otherwise prejudicially change or alter the surfaces. If the comminution is effected in the presence of water, as in the ball mill, the water serves as a protective agent as against alteration for a considerable time, and a similar temporary protection would be afforded by wetting coal that has been comminuted in the dry state. Apparently, killing of the luster of the surfaces of the

coal particles is due to oxidation thereof, and it should usually be guarded against in the practice of the invention, to obtain the best results.

What I claim is:

1. The method of concentrating bituminous coal, which comprises comminuting the bituminous coal to produce a finely divided product with particles having sharp angular edges and fresh lustrous surfaces, and subjecting the resulting product to separation by froth flotation. 30

2. The method of concentrating coal which comprises comminuting bituminous coal washer refuse to produce a finely divided product with particles having sharp angular edges and fresh lustrous surfaces, 35 and subjecting the resulting product to separation by froth flotation. 40

In testimony whereof I affix my signature.

RAYMOND F. BACON.